

Feb. 4, 1964

G. B. HATCH

3,120,425

ZINC SILICOFLUORIDE COMPOSITION AND  
METHOD OF PREVENTING CORROSION

Filed March 28, 1962

4 Sheets-Sheet 1



INFLUENCE OF pH ON THE CORROSION OF STEEL AT  
SEVERAL ZINC SILICOFLUORIDE CONCENTRATIONS.

FIG. 2



INFLUENCE OF Zn<sup>2+</sup>-SiF<sub>6</sub><sup>-2</sup> RATIO ON THE  
CORROSION OF STEEL (pH 6.5).

FIG. 1

INVENTOR  
GEORGE B. HATCH

BY

William L. Krayer,  
ATTORNEY

Feb. 4, 1964

G. B. HATCH  
ZINC SILICOFLUORIDE COMPOSITION AND  
METHOD OF PREVENTING CORROSION

3,120,425

Filed March 28, 1962

4 Sheets-Sheet 2



ZnSiF<sub>6</sub> · 6H<sub>2</sub>O CONC. - P.P.M.  
INFLUENCE OF ZINC SILICOFLUORIDE  
CONCENTRATION ON THE CORROSION OF COPPER.

FIG. 4



ZnSiF<sub>6</sub> · 6H<sub>2</sub>O CONC. - P.P.M.  
INFLUENCE OF ZINC SILICOFLUORIDE CONCENTRATION ON  
THE CORROSION OF STEEL AT SEVERAL pH LEVELS.

FIG. 3

INVENTOR

GEORGE B. HATCH

BY

William L. Krayer.  
ATTORNEY

Feb. 4, 1964

G. B. HATCH

3,120,425

ZINC SILICOFLUORIDE COMPOSITION AND  
METHOD OF PREVENTING CORROSION

Filed March 28, 1962

4 Sheets-Sheet 3



INFLUENCE OF ZINC SILICOFLUORIDE CONCENTRATION  
ON THE CORROSION OF STEEL IN THE PRESENCE  
OF 5 P.P.M. SODIUM DICHROMATE. FIG. 5

FIG. 6

Zn<sub>2</sub>SiF<sub>6</sub> · 6H<sub>2</sub>O CONC. - P.P.M.  
INFLUENCE OF ZINC SILICOFLUORIDE CONCENTRATION  
ON THE CORROSION OF STEEL IN THE PRESENCE  
OF 5 P.P.M. SODIUM DICHROMATE. FIG. 6

INVENTOR  
GEORGE B. HATCH

BY

William L. Krayer.  
ATTORNEY

Feb. 4, 1964

G. B. HATCH  
ZINC SILICOFLUORIDE COMPOSITION AND  
METHOD OF PREVENTING CORROSION

3,120,425

Filed March 28, 1962

4 Sheets-Sheet 4



EFFECT ON GALVANIC ATTACK OF COPPER  
AND STEEL IN SOLUTIONS OF ZINC AND  
CHROMATE INHIBITORS CONTAINING VARYING  
AMOUNTS OF  $\text{SiF}_6^-$ .

INVENTOR.  
GEORGE B. HATCH  
BY

FIG. 7

William L. Krayev.  
ATTORNEY

## 1

3,120,425

ZINC SILICOFLUORIDE COMPOSITION AND  
METHOD OF PREVENTING CORROSION  
George B. Hatch, Allison Park, Pa., assignor to Calgon  
Corporation, a corporation of Pennsylvania  
Filed Mar. 28, 1962, Ser. No. 183,291  
9 Claims. (Cl. 21—2.7)

This invention relates to inhibiting the corrosion of metals in contact with water. In particular, it relates to the use of zinc silicofluoride to inhibit the corrosion of metals in contact with aqueous media such as industrial waters.

It is known to those skilled in the art of corrosion inhibiting that most commercial corrosion inhibitors exhibit one or more undesirable characteristics wholly apart from their abilities to inhibit corrosion. One of these weaknesses is a susceptibility to destruction by oxidizing or reducing agents present in the system. Another is the tendency of some corrosion inhibitors to encourage the growth of biological organisms because of their nutrient properties. Other corrosion inhibitors have the undesirable trait of depositing a relatively permanent stain on susceptible surfaces. I have invented methods and compositions which are excellent for inhibiting corrosion of metals and at the same time are not undesirable because of any of the above traits.

I have discovered that zinc silicofluoride ( $ZnSiF_6$ ) provides surprisingly good corrosion inhibition in aqueous systems such as in cooling towers and other industrial waters, by itself or in combination with other corrosion inhibitors.

The accompanying seven figures illustrate the effectiveness of my invention. FIGURE 1 is a plot of the corrosion inhibition curve of various concentrations of zinc ion and silicofluoride ion, showing the synergistic action at the ratio of zinc silicofluoride. FIGURE 2 is a graph of the influence of pH on the corrosion inhibiting action of zinc silicofluoride. FIGURE 3 is a different view of the same points plotted in FIGURE 2 to, clearly illustrate the effect of pH. FIGURE 4 shows the corrosion inhibiting effect of zinc silicofluoride on copper. FIGURE 5 illustrates the effect of my invention in the presence of "Calgon" brand sodium hexametaphosphate. FIGURE 6 depicts the effect of zinc silicofluoride in the presence of still another known corrosion inhibitor, sodium dichromate. FIGURE 7 plots the effect on galvanic attack of increasing concentrations of silicofluoride ion.

The weight loss data in the drawings were obtained from agitated batch tests in 1 liter of a water closely approximating an average analysis of Pittsburgh tap water. The water used in all demonstrations recited herein contained 19 p.p.m. calcium, 6.0 p.p.m. magnesium (hardness thus calculated as 77 p.p.m.  $CaCO_3$ ), 18 p.p.m. chlorine, and 12 p.p.m.  $HCO_3$ . The tests were run for five days at 35° C.  $\pm 0.1^\circ$ . The concentrations of zinc silicofluoride in all figures except FIGURE 1 are calculated as the hexahydrate and represent concentrations of zinc silicofluoride hexahydrate.

FIGURE 1 illustrates that the action of zinc silicofluoride is not merely an additive effect of its ionic components. The  $SiF_6^{2-}$  ion alone is practically ineffective. Although the zinc ion alone has some inhibiting effect, it cannot compare with the results obtained when the zinc ions are in the presence of silicofluoride ion. If the effect were merely additive, one would expect a mixture of 50 p.p.m. zinc and 50 p.p.m. silicofluoride ion to result in a loss of about 80 mg./sq. decimeter/day. As can be seen in FIG. 1, the loss is rather only about 4 mg./sq. decimeter/day.

FIG. 2 records the weight loss in milligrams per square decimeter per day of steel immersed in water containing

## 2

various concentrations of zinc silicofluoride. It will be seen that even in concentrations over 50 p.p.m., zinc silicofluoride alone does not provide startlingly effective inhibition at a pH less than 6 although it does exhibit an inhibiting effect. It is strikingly effective at pH's above 6 as can be seen from the graph of FIG. 2.

The same points of FIG. 2 are presented differently in FIG. 3 to emphasize the effect of pH. Although some inhibition is provided at pH 5, it is preferred to use my invention at a pH of at least 6. Preferably it will be used at a pH no higher than 8 because of the danger of precipitating zinc compounds at higher levels. As little as 5 p.p.m. of zinc silicofluoride will provide a noticeable inhibiting effect; however, it is preferred to use at least about 10 p.p.m. of zinc silicofluoride hexahydrate or the equivalent less hydrous compound.

That my invention also has an excellent inhibitive effect on the corrosion of copper is shown in FIG. 4. Again, a pH of 8 is considered the maximum practical limit because of precipitation problems.

A striking effect is produced by the use of zinc silicofluoride in the presence of sodium hexametaphosphate to inhibit the corrosion of steel. FIG. 5 compares the inhibiting effect of zinc silicofluoride in various concentrations in the presence of "Calgon" brand sodium hexametaphosphate at a strength of ten parts per million. The pH at each test was 6.5, but may vary between the limits of about 5 and 8 as suggested elsewhere herein.

FIG. 6 is a similar graph illustrating the striking effect 30 of a combination of zinc silicofluoride and sodium dichromate. Again, the pH of the tests was 6.5, but it may vary between about 5 and about 8. An outstanding advantage of the use of zinc silicofluoride together with sodium dichromate over sodium dichromate alone is that 35 the inhibiting effect will be substantially preserved during periods when the dichromate may be subject to severe reduction.

FIG. 7 demonstrates the effect of my invention on galvanic corrosion. In this demonstration, a test panel of 40 copper and one of steel 1½" square were immersed in parallel planes at a distance of ½ inch in water containing various concentrations of  $SiF_6^{2-}$  ion and zinc ion as noted. Electrode leads were connected to the panels; the current generated as measured in milliamperes is plotted 45 against time on the graph. The five solutions shown on the graph as 0%, 25%, 50%, 75%, and 100% contain varying proportions as noted on  $SiF_6^{2-}$ . They were prepared from two solutions, one representing 100%  $SiF_6^{2-}$  (a 37½ p.p.m. solution of a composition consisting of 50 20% sodium-dichromate dihydrate and 80% zinc silicofluoride hexahydrate) and the other representing 0%  $SiF_6^{2-}$  (25 p.p.m. of a mixture of 70%  $ZnSO_4 \cdot H_2O$  and 30%  $Na_2Cr_2O_7 \cdot 2H_2O$ ). The solution marked 50% on the graph had ½ the amount of  $SiF_6^{2-}$  in the 100% solution. It 55 was prepared by mixing 12 parts by weight of the 0% composition and 18¾ parts by weight of the 100% composition. The 25% and 75% solutions were made in a similar manner from the 0% and 100% compositions. Each solution thus contained the same amount of zinc and chromate ions, and in the same ratio of 1:1. As the amount of zinc silicofluoride was reduced in each successive solution, the amount of zinc introduced through zinc sulfate was increased. Thus the 25% solution contained 3.4 p.p.m. of  $SiF_6^{2-}$ , the 50% solution contained 6.8 p.p.m. of  $SiF_6^{2-}$ , the 75% solution contained 10.2 p.p.m. of  $SiF_6^{2-}$ , and the 100% solution contained 13.5 p.p.m. of  $SiF_6^{2-}$ , while the zinc and chromate remained substantially constant.

The compositions used in the demonstrations recorded 70 in FIG. 7 are not limited in effect to the inhibition of galvanic attack but are also effective in aqueous systems containing only one metal.

In addition to the corrosion inhibiting effects illustrated in the graphs, the combination of zinc silicofluoride with sodium hexametaphosphate or sodium dichromate (or both) provides the system with stabilization of aluminum. Aluminum may be present in a water system as a carry-over from clarification processes, and is undesirable where corrosion is likely to occur.

The maximum amount of zinc silicofluoride which may be of use is governed only by economics and solubility factors. In many industrial waters, up to 500 p.p.m. of zinc silicofluoride may be carried without precipitation. When other inhibitors are present, such as sodium hexametaphosphate or sodium dichromate, a safe practical limit is about 200 p.p.m. of zinc silicofluoride. The maximum amount of other inhibitors is generally unaffected by the presence of zinc silicofluoride. For example, the teachings of Rice and Hatch, U.S. Patent 2,337,856, may be followed with regard to effective amounts of sodium hexametaphosphate. Chromates and dichromates may be used in large concentrations with zinc silicofluoride. However, it is preferred to use chromates and dichromates in the presence of additional zinc ions according to the teachings of my U.S. Patent 3,022,133. Zinc silicofluoride may be combined, within the scope of the present invention, with both a chromate (with or without a separate source of zinc as in U.S. Patent 3,022,133) and a phosphate glass.

A preferred composition employing zinc silicofluoride and sodium dichromate, as suggested in the demonstration of FIG. 7, consists essentially of 35% by weight of zinc sulfate monohydrate, 40% zinc silicofluoride hexahydrate, and 25% sodium dichromate. Of course, zinc silicofluoride may be used with combinations of the zinc and  $\text{Cr}_2\text{O}_7$  ion in other ratios. It may be incorporated in any composition providing dichromate ions with or without additional zinc ions. The use of such combinations may be expressed as a method of treating aqueous media to inhibit corrosion of metals in contact therewith comprising adding to such media (a) at least about five parts of zinc silicofluoride (calculated as the hexahydrate) per million parts of water, (b) at least one water soluble zinc salt, such as zinc sulfate, zinc chloride, zinc nitrate, and similar zinc salts capable of producing up to about 10 p.p.m. zinc ions under the conditions present, and (c) sufficient water-soluble chromate and/or dichromate compounds to produce up to about 25 p.p.m. chromate and/or dichromate ions.

As little as 10 p.p.m. or less of a composition of 8 parts by weight zinc silicofluoride hexahydrate, 7 parts by weight zinc sulfate monohydrate, and 5 parts by weight sodium dichromate produces good corrosion inhibiting results in most industrial waters, although the optimum range is considered to be about 25-50 p.p.m., preferably in a solution having a pH in the optimum range of 6.5-7.2.

From the foregoing figures and data, it will be seen that zinc silicofluoride is an effective corrosion inhibitor by itself in aqueous systems of pH about 5 to about 8 in concentrations of at least about 5 p.p.m. As is indicated in the figures, even less than 5 p.p.m. of zinc silicofluoride in the presence of known corrosion inhibitors will enhance the effect thereof. As can be seen from FIG. 5, as little as 1 p.p.m. of zinc silicofluoride reduces weight loss to less than half that resulting from the use of 10 p.p.m. sodium hexametaphosphate alone.

Zinc silicofluoride ( $\text{ZnSiF}_6$ ) is very difficult to oxidize

or reduce. Consequently, it is stable to oxidizing agents including those normally found in industrial water, such as chlorine. At the same time it is highly resistant to reduction by reducing agents occasionally found in water, such as organic matter, sulfur dioxide, and so forth. It will not serve as a nutrient for algae or slime bacteria. Since it is colorless, it causes no staining problems.

Having thus described and illustrated certain presently preferred embodiments of my invention and methods of practicing the same, it is to be distinctly understood that it is not limited thereto but may be otherwise variously embodied and practiced within the scope of the following claims.

I claim:

- 15 1. Method of inhibiting the corrosion of metals in contact with water comprising adding to said water at least about 5 p.p.m. of zinc silicofluoride calculated as the hexahydrate and maintaining the pH between about 5 and about 8.
- 20 2. Method of inhibiting the corrosion of metals in contact with water comprising adding to said water an effective amount of zinc ions and  $\text{SiF}_6^{2-}$  ions and maintaining the pH between about 5 and about 8.
- 25 3. Method of inhibiting the corrosion of steel in contact with water comprising adding to the water a small amount of zinc silicofluoride and a small amount of sodium hexametaphosphate.
- 30 4. Method of inhibiting the corrosion of steel in contact with water comprising adding to the water at least about 5 p.p.m. of zinc silicofluoride and a small amount of sodium dichromate.
- 35 5. A composition useful in inhibiting the corrosion of metals in aqueous systems comprising sodium hexametaphosphate and zinc silicofluoride.
- 40 6. A composition useful in inhibiting the corrosion of metals in aqueous systems comprising sodium dichromate and zinc silicofluoride.
- 45 7. A composition useful in inhibiting the corrosion of metals in aqueous systems comprising sodium dichromate, sodium hexametaphosphate, and zinc silicofluoride.
- 50 8. A composition useful in inhibiting corrosion in aqueous systems comprising
  - (a) zinc silicofluoride,
  - (b) a water-soluble zinc salt,
  - (c) a water-soluble compound capable of producing in solution an anion of the group consisting of chromate ion and dichromate ion.
- 55 9. Method of inhibiting the corrosion of metals in contact with aqueous media comprising adding to said aqueous media
  - (a) at least about 5 parts per million of zinc silicofluoride,
  - (b) about 2 to about 10 parts per million of additional zinc ion, and
  - (c) up to about 25 parts per million of an ion from the group consisting of chromate ion and dichromate ion.

References Cited in the file of this patent

UNITED STATES PATENTS

|           |               |                |
|-----------|---------------|----------------|
| 2,719,079 | Murphy        | Sept. 27, 1955 |
| 2,848,299 | Kahler et al. | Aug. 19, 1958  |
| 2,900,222 | Kahler et al. | Aug. 18, 1959  |
| 3,010,854 | Satterfield   | Nov. 28, 1961  |